

Patented June 26, 1928.

1,674,955

# UNITED STATES PATENT OFFICE.

REGINALD SCOTT DEAN AND WILLIAM EWART HUDSON, OF OAK PARK, ILLINOIS, AS  
SIGNORS TO WESTERN ELECTRIC COMPANY, INCORPORATED, OF NEW YORK, N. Y.,  
A CORPORATION OF NEW YORK.

## PROCESS FOR PREPARING LEAD ALLOYS ON WHICH WORK IS TO BE PERFORMED.

No Drawing.

Application filed February 5, 1924. Serial No. 690,717.

This invention relates to a process for preparing lead alloys on which work is to be performed.

An object of this invention is to provide a process for preparing lead alloys on which work is to be performed whereby said work may be more easily, feasibly and efficaciously accomplished.

Another object of this invention is to provide a process for working lead alloys more quickly and with less incidental delay than has heretofore been possible.

A further object of this invention is to provide a process for forming lead antimony articles of higher antimony content than has heretofore been possible with out the development of blisters, fractures, or other similar irregularities.

In describing the process which is the basis of this invention reference will be made to the extrusion of cable sheath, but it is to be understood that the process of preparing the alloy can be efficiently employed whenever work of any type is employed to produce a lead alloy article.

Heretofore the process used for extruding lead alloys has been as follows: The required proportions of lead and alloying matter were melted in a kettle or melting pot. The molten lead alloy was then introduced into the cylinder of an extruding press, where it was allowed to solidify, the time required for solidifying being in practice between six and ten minutes. As soon as the lead had solidified, it was extruded into the form desired. As an alternative the ingot was cast outside of the press and subsequently introduced into the press cold and extruded after it has been heated up in the press cylinder. For fast extrusion it is necessary to work at as high a temperature as possible. It is known that the plasticity of a metal is approximately doubled for a 10° C. rise in temperature. It follows that the rate of extrusion with a given pressure and orifice will be approximately doubled by a 10° C. rise of temperature. The advantage of using the highest possible temperature is, therefore, clear. In lead presses when the extrusion temperature was raised to permit more rapid extrusion, certain defects such as blisters, cracks, splits, and the like were encountered in the sheath formed. These defects are encountered more frequently when

the content of antimony or other alloying element is increased.

It is known that when an alloy of lead and antimony is cast and rapidly cooled that the resulting alloy has areas of eutectic alloy and that as the antimony increases, these areas increase. It is reasonable to suppose that the defects referred to are caused at least in part by the presence of these eutectic areas, since the eutectic becomes molten at a temperature below that of the remainder of the alloy.

Attempts have been made to increase the percentage of antimony in lead-antimony alloys. Such increase has had the effect of developing eutectic areas, which, it is supposed, cause the imperfections which appear on the extruded article. An attempt was made to extrude at a lower temperature, but difficulty was again experienced, due, it seems, to insufficient plasticity at temperatures below the eutectic melting temperature.

It was established in the investigation on which this invention is based that the solid solubility of antimony in lead at room temperature is approximately 1 per cent, and increases with the increases of temperature. At 240° C., which is slightly below the eutectic fusing temperature, the solubility is about 2.5%. By heating ingots of lead-antimony alloys containing less than 3 per cent antimony for a sufficient length of time, it was found that a homogeneous solid solution could be formed, the eutectic areas disappearing. For a more detailed description of a process for forming solid solutions of lead and antimony our co-pending application, Serial No. 690,716, filed February 5, 1924, may be referred to.

Based on this discovery the process hereinafter described of extruding lead alloys has been developed. In carrying out this invention an ingot of lead-antimony alloy is cast, and then heated or soaked for a period of time before extrusion. The ingot can then be placed in an extruding press and extruded at a higher temperature, and consequently with greater celerity, without any apparent irregularities being developed. The time formerly required for the molten lead to solidify in the press cylinder is also saved, the extrusion being almost continuous. In addition this heating or soaking treatment will allow the use of an alloy having a greater

antimony content, without the difficulties experienced in the use of that same alloy under the old method. A study of the article extruded from such a soaked or annealed ingot 5 shows a disparity or total absence of eutectic areas.

Specifically a method employed in the extrusion of cable sheath is as follows: the ingot is cast outside of the extruding press and 10 subsequently placed in an oven in which a temperature of 240° C. is maintained for 72 hours.

After this heating or soaking, the ingot is placed in an extruding press and immediately extruded. Immediate extrusion is not 15 necessary, however, since if the ingot is once heated for a sufficient length of time, it may be cooled and then by reheating for a comparatively short length of time, it may 20 be used equally well. Good results may be obtained by varying the time and temperature of heating somewhat. The specific process above described has been adopted because universally good results seem to be obtained by it. 25

The explanation of the lack of eutectic areas in the cable sheath by means of this process and the coincident fact that such cable sheath shows none of the irregularities, 30 such as blisters, cracks, or fractures, which appear in articles extruded under the old process, would seem to lie in the discovery that the solid solubility of the lead in antimony varies with the temperature of the 35 alloy. It would seem that an annealing process gradually allows the proportion of antimony in solution in the lead to increase until the maximum amount at the given temperature is reached.

This explanation is apparently borne out 40 in the fact, since, as heretofore noted, eutectic areas are not noticed on the cable sheath extruded from the heated slug.

The process above described facilitates 45 quick extrusion by reason of the fact that the operation may be carried on at a comparatively high temperature. In addition it allows more continuous extrusion by obviating the objectionable feature of having to 50 wait for a length of time for the lead to solidify, (6 minutes being the average) or for a cold ingot to be heated before extrusion can be continued.

This process can be used in preparing any 55 lead alloys for extrusion. A high tin content, lead tin alloy, for instance, may be extruded much more efficiently by the use of this method.

Wherever alloying matter is used which 60 forms a homogeneous solution, mixture, or compound with the lead rather slowly, and which forms such a solution, mixture or compound better at a higher temperature, this 65 method has a beneficial use. This invention is present in any process where lead alloy is

cast and then heated for a period of time before being worked.

What is claimed is:

1. A process for preparing lead alloys on which work is to be performed, which consists in casting an ingot of the alloy, and then by heating reducing said alloy to a substantially homogeneous solid solution. 70

2. A process for preparing lead-antimony alloys for extrusion, which consists in casting the alloy and heating said alloy at a temperature of 240° C. until a solid solution is formed, said solid solution containing substantially all of the antimony present in the alloy. 75

3. A process for preparing lead-antimony alloys for extrusion, which consists in casting an ingot containing not more than 3% antimony, and heating said ingot at a temperature of 240° C. for about 72 hours. 80

4. A process for extruding lead-antimony alloys, which consists in initially casting an ingot, and heating said ingot at 240° C. for about 72 hours, placing said slug in an extruding press, and extruding. 85

5. A process for extruding lead-antimony alloys containing up to 3 per cent antimony, which consists in casting an ingot of said alloy, heating said ingot until a substantially homogeneous solid solution is formed, placing said ingot in an extruding press, and extruding. 90

6. A process for extruding lead alloys, which consists in casting an alloy ingot, forming said ingot into a solid solution by 100 heating, and extruding.

7. A process for preparing lead alloys on which work is to be performed, which consists in casting the alloys in the form of an ingot, and then heating said ingot at a temperature slightly below the fusion temperature until a substantially homogeneous solid solution is formed, said solid solution containing substantially all of the solute material present in the alloy. 105

8. A process for preparing lead-antimony alloys for extrusion, which consists in casting an ingot of the alloy, and heating said ingot at a temperature slightly below the fusion temperature until a substantially homogeneous solid solution is formed, said solid solution containing substantially all of the antimony present in the alloy. 115

9. A process for preparing lead-antimony alloys for extrusion, which consists in casting an ingot of an alloy containing about 2.5% antimony, and heating said ingot at a temperature slightly below the fusion temperature for about 72 hours. 120

In witness whereof, we hereunto subscribe our names this 22nd day of January A. D. 1924.

REGINALD SCOTT DEAN.  
WILLIAM EWART HUDSON.